

Patented May 12, 1925.

## UNITED STATES PATENT OFFICE.

HUGH C. SICARD, OF NEW YORK, N. Y.

## PROCESS OF REMOVING NONMETALLIC INCLUSIONS FROM IRON OR STEEL.

No Drawing.

Application filed November 1, 1923. Serial No. 672,177.

*To all whom it may concern:*

Be it known that I, HUGH C. SICARD, a citizen of the United States of America, and a resident of the city of New York and State of New York, have invented a certain new and useful Process of Removing Non-metallic Inclusions from Iron or Steel, of which the following is a full, clear, and exact description.

10 In general my process relates to a method of removing any non-metallic inclusions from iron or steel, and in particular it relates to a method of removing the oxides of metals from iron or steel.

15 It is the common practice of the art in making steel or ingot iron of any low carbon content to oxidize the carbon in a basic open-hearth furnace or in an electric furnace until the percentage has reached the desired amount. This practice inevitably results in the formation of oxides of metals, that is, non-metallic inclusions in the iron or steel. These oxides affect the properties of the iron and steel adversely, and as a consequence it has been the practice to use more or less aluminum as the deoxidizer, since the aluminum reacts with the oxides in the molten metal. In adding the aluminum as a deoxidizer the iron or steel is tapped into a receiving ladle, and the aluminum is added thereto. The aluminum immediately reacts with the various oxides suspended in the steel, thus forming alumina, which, as is well known, is an extremely refractory oxide, and quite infusible at the temperature of molten steel. A result of this treatment is that the alumina derived from the aluminum, which has been used as a deoxidizer, will be entrapped in the steel or iron during its solidification in the molds, and will thus affect adversely the physical properties of such iron or steel.

By means of experiments, I have found that titanic oxide is a suitable fluxing agent for alumina. Thus I have found that titanic oxide and alumina, when heated together form a much more fusible compound than is the alumina, and in the form either of artificially made oxide or as the natural titanic oxide, rutile, forms a cheaper and effective flux. I have found that in a wide range of proportions, the combination of titanic oxide and alumina forms a low melting point compound, and, therefore, the addition of titanic oxide to molten steel or iron containing alumina forms a slag of the

latter which easily separates from the metal, thus avoiding objectionable inclusions in it. My invention consists in the use of titanic oxide in any of its forms, natural or artificial, as an addition to a bath of molten iron or steel with the object of fluxing the alumina produced by the use of aluminum as a deoxidizer.

In carrying out my invention, I employ a furnace of any suitable type in which is formed a molten bath of metal. When the furnace is tapped into the ladle, I throw in titanic oxide and it melts rapidly. When the ladle is about half or three-fourths full, the deoxidizing aluminum is added to the bath. The aluminum is immediately oxidized, and the alumina thus produced fluxes with the titanic oxide, thus producing an iron or steel free from any inclusions. Not only does the titanic oxide flux the alumina but it also combines with other oxides such as lime or the like.

While the foregoing describes the usual method of carrying out my process, it should be noted that without departing therefrom the aluminum may be added to the ladle first and later the titanic oxide may be added, or both the aluminum and the titanic oxide may be added simultaneously.

Having thus described my invention, what I claim is:

1. A process of removing non-metallic inclusions from iron or steel comprising the formation in a suitable furnace of a molten bath of iron or steel, then tapping the furnace into a ladle, then adding to the contents of the ladle titanic oxide, and then adding to the contents of the ladle alumina.

2. A process of removing non-metallic inclusions from iron or steel comprising the formation in a suitable furnace of a molten bath of iron or steel, then tapping the furnace into a ladle, then adding to the contents of the ladle aluminum, and then adding to the contents of the ladle titanic oxide.

3. A process of removing non-metallic inclusions from iron or steel comprising the formation in a suitable furnace of a molten bath of iron or steel, then tapping the furnace into a ladle, and then simultaneously adding to the contents of the ladle titanic oxide and aluminum.

In testimony whereof, I have hereunto signed my name.

HUGH C. SICARD.